

# UNITED STATES PATENT OFFICE.

GEORGE A. GOODSON, OF MINNEAPOLIS, MINNESOTA.

## PLATED METALLIC BODY.

No. 900,846.

Specification of Letters Patent.

Patented Oct. 13, 1908.

Application filed March 28, 1906. Serial No. 308,445.

*To all whom it may concern:*

Be it known that I, GEORGE A. GOODSON, a subject of the King of Great Britain, residing in Minneapolis, Hennepin county, Minnesota, have invented certain new and useful Improvements in Plated Metallic Bodies; and I do hereby declare the following to be a full, clear, and exact description of the invention, such as will enable others skilled in the art to which it appertains to make and use the same.

My invention relates to that class of metallic bodies which are protected against corrosion under the action of the elements, as, for example, those in the air or in water, by metallic plating; and has for its object to provide an improved product or article of manufacture of this general class. Hitherto, as is well known, it has been the common practice to galvanize or plate metallic bodies, such, for example, as iron and steel wire, or iron or steel sheets or plates, with zinc as the plating metal, or with an alloy composed of about one-third tin and two-thirds lead; and this plating has been done by submerging the wire or other metallic body in the said classes of molten plating metal at the proper temperature.

Zinc or an alloy of tin and lead, such as above stated, (owing to the presence of the tin therein), have such great affinity for iron or steel that such plating metals can be made to adhere to wire or steel metallic bodies by said old process above indicated. Zinc is a hard and brittle metal; and, when used for plating purposes, is apt to crack and scale should the wire or other plated body be twisted, hammered, or otherwise distorted; and to minimize this tendency to crack or scale, it has, in practice, been found necessary to apply only a very thin coating or plating of the zinc to the wire or other metallic body. In this effort to employ only a thin coating of zinc, the metallic body so plated is frequently left uncovered in places, which, of course, renders the plated body much more liable to deterioration by corrosion under the action of the elements; and, moreover, such extremely thin plating soon deteriorates from corrosion.

The above stated alloy of tin and lead can be applied to the wire or other metallic body in a thicker coat, because such alloy is much less brittle than zinc. Tin, however, rapidly deteriorates from the corrosion incidental to the action thereon of the elements

in the air or water, and to which the wire or other body plated therewith is necessarily exposed in the service; and tin has thus been employed hitherto with the lead, simply because of its known affinity for iron or steel; or otherwise stated, the alloy could be made to adhere to the plated body and lead could not.

It has long been known that lead would be the ideal plating metal, because of its pliability and its non-corrodibility under the action of the elements to which such body must be exposed in actual service; but prior to the invention or discovery made by me, and disclosed in my U. S. Patent No. 789,690, of date May 9th, 1905, it had never been found commercially practicable to plate metallic bodies with lead. Lead has so little affinity for other metallic bodies like iron and steel, that, under the old process, which was satisfactory for plating with zinc, or with the above stated alloy of tin and lead, the lead could not be made to adhere to the plated body. Under my said process, disclosed in my said patent, I have found that iron and steel bodies can be plated with pure lead, and that the union is so close as to permanently unite the two metals. By reference to my above identified patent, it will be seen that I accomplish this result by subjecting the wire or other metallic body to be plated to a bath of molten plating metal, which has been subjected to an electric current of the proper strength, while the said plating metal was in molten condition. In my actual practice, I have ordinarily employed a current of from 1500 to 2000 amperes for a cross section of one inch. The body to be plated is, of course, cleaned by pickling the same in the usual way before it is submerged in the molten bath of the plating metal.

I have plated considerable quantities of iron and steel wire with pure lead as the plating metal, under my said process above noted, and have also plated considerable quantities of iron and steel sheet metal with pure lead, under my said process, and I have found that the union between the particles of the plated body and the lead is so close that the lead will not scale, crack, or break even when the wire or other plated body is twisted, hammered, or drawn. If the plating metal has been properly treated with the electric current, it appears to be a matter of indifference whether the current is on or off

when the actual plating is done. I have also secured the same general result with the use of an alloy containing chiefly lead, but a small percentage of antimony. As is well known, antimony has a hardening effect in such an alloy with lead. As above stated, lead is the ideal metal for plating, so far as its ductility and non-corrodibility is concerned; and the only objection there is to the use of pure lead is that it is a little too soft, and will wear away under some classes of service where it is liable to abrasion from any cause. By the addition of a small percentage of antimony, to wit, about 13 percent. to the 87 percent. of lead, I get an alloy having all the required properties of pliability, and non-corrodibility necessary for good commercial service, while, at the same time, the requisite hardness is present to prevent the ready wearing away from abrasion. The presence of this small quantity of antimony does not appear to in any wise diminish or impair the closeness of the union which takes place between the particles of the plating metal and the body to be plated, when the plating is done under my process above pointed out. So far in my practice, I have only tried out antimony as the harden-

ing metal to use in connection with lead, but it is probable that some other hardening metals, such as arsenic, might possibly be used, and hence I do not limit myself, in a broad point of view, solely to use of antimony as the hardening element.

Having thus described my invention, what I claim and desire to secure by Letters Patent, is:—

1. As a new article of manufacture, a metallic body plated with an alloy composed chiefly of lead but containing a small percentage of some hardening metal, which alloy has been subjected to an electric current while in molten condition.

2. As a new article of manufacture, a metallic body plated with an alloy composed chiefly of lead but containing a small percentage of antimony, which alloy has been subjected to an electric current while in a molten condition.

In testimony whereof I affix my signature, in presence of two witnesses.

GEORGE A. GOODSON.

Witnesses:

JAS. F. WILLIAMSON,  
EDWIN S. CLARKSON.